

Sept. 10, 1940.

E. H. GREENBERG

2,214,611

APPARATUS FOR TREATING METALS

Filed Dec. 16, 1936

3 Sheets-Sheet 1



INVENTOR

Elmer H. Greenberg

BY

Ward, Conley & Neal

ATTORNEY

Sept. 10, 1940.

E. H. GREENBERG

2,214,611

APPARATUS FOR TREATING METALS

Filed Dec. 16, 1936

3 Sheets-Sheet 2



Sept. 10, 1940.

E. H. GREENBERG

2,214,611

## APPARATUS FOR TREATING METALS

Filed Dec. 16, 1936

3 Sheets-Sheet 3

Fig. 6.



Fig. 7.



INVENTOR  
Elmer H. Greenberg  
BY  
Ward, Cough & Neal  
ATTORNEY

## UNITED STATES PATENT OFFICE

2,214,611

## APPARATUS FOR TREATING METALS

Elmer H. Greenberg, Philadelphia, Pa.

Application December 16, 1936, Serial No. 116,139

9 Claims. (Cl. 266—34)

This invention relates to an apparatus and process for treating metals and particularly for detinning lead alloys. It is especially concerned with such apparatus and process for the production and removal of tin as volatile tin tetrachloride from alloys or mixtures containing lead and tin.

It is known that chlorine gas will react with lead and tin to form lead chloride and stannous chloride. Stannous chloride in the presence of more chlorine is changed into stannic chloride which is volatile at a known elevated temperature and by heating to that temperature should theoretically be removable from the lead chloride which is not volatile when heated to that temperature. Apparatuses and processes have been heretofore proposed utilizing this principle for separation of tin, but various difficulties have been encountered due in part to lack of appreciation of the proper conditions for operation and in part to the highly corrosive and poisonous nature of chlorine gas, particularly at high temperatures. The use of chlorine on mixtures of alloys containing lead and tin at low temperatures where the metal is in granular but not melted state, is not practical because the chlorine attacks the exterior of the granules but the chlorides formed then prevent contact of the chlorine with the metals underneath. Operation at higher temperatures has not been practical prior to the present invention, so far as I am aware, because of difficulties in providing a suitable apparatus and process that could be operated economically and efficiently to produce the desired results.

The principal object of my invention accordingly is to overcome at least some of the difficulties heretofore recognized and to provide a practical apparatus and process for the desired removal of tin from mixtures or alloys containing lead and tin with or without other metals.

The invention accordingly comprises the novel apparatus and combinations thereof, as well as the novel processes and steps of processes which may be carried out in such apparatus, specific embodiments of which are described herein by way of example only and in accordance with the manner in which I now prefer to practice the invention.

In the accompanying drawings in which are shown embodiments of the apparatus as I now prefer it,

Fig. 1 is a diagrammatic elevation partly in section of the apparatus;

Fig. 2 is an enlarged detail section of the reaction chamber;

Fig. 3 is a cross-section thereof on the line 3—3 of Fig. 2;

Fig. 4 is an enlarged detail view of one of the 5 plurality of chlorine pipes passing from a bustle pipe into the reaction chamber;

Fig. 5 is a diagrammatic view partly in section of a modification of the kettle and reaction chambers in which two kettles are employed provided 10 so that a constant level of molten metal may be maintained easily in the kettle in which the reaction chamber is placed;

Fig. 6 is a diagrammatic elevation partly in section of another modification of the apparatus showing three kettles permitting continuous operation of the process; and

Fig. 7 is a diagrammatic elevation partly in section showing a modification of the apparatus shown in Fig. 5 and in place of the second kettle employing a furnace with a bay in which the pump works. 20

Because of the corrosive and poisonous character of chlorine, especially at temperatures of 1000°—1050° F. at which I prefer to practice the 25 process of the invention as described below, I have shown in the drawings an apparatus in which the chlorine, while combining with the tin, operates in a comparatively restricted area. In that area the apparatus is preferably lined with 30 a chlorine-resistant material which is described and claimed in my copending application Ser. No. 120,877, filed January 16, 1937. In addition the chlorine is confined within this area so that its 35 escape beyond it in any substantial quantity is prevented. If small quantities pass off with the volatilized tin chloride they are collected by washing, as later described.

Referring now to the drawings and particularly to Figs. 1 to 4, the numeral 1 designates 40 an open steel kettle supported in a kettle setting 2. 3 is a burner which may be operated by oil or gas and passes through a port in the kettle setting in order to heat the kettle 1. 4 is a framework of channel iron or similar structure 45 extending across the top of the kettle to support the reaction chamber and other apparatus hereinafter described. 5 is an electric motor mounted on the channel iron 4 and serving to operate the pump 6. This pump per se is described and 50 claimed in my copending application Ser. No. 118,704, filed January 2, 1937. The pump is connected by pipe 7 with a cylindrical reaction chamber open at the bottom, which has an outer shell of cast iron 8 lined on the inside with 55

clay brick 9 (see Figs. 2 and 3). Inside the clay brick 9 is a special concrete layer 10 adapted to withstand the corrosive effects of chlorine at the temperatures above mentioned. This concrete is that referred to in my copending application Ser. No. 120,877 above, and is composed of crushed fire brick, Portland cement with high alumina content and sand. This cement as shown protects the various parts of the apparatus which it surrounds from the corrosive action of the chlorine gas and molten chloride. The pipe 7 it will be noted passes through the top of this reaction chamber and terminates a little below the top of the reaction chamber 15 passing through the cement 10 and discharging into a substantially cylindrical space about the center of the reaction chamber, into which space stannic chloride rises on its way out of the reaction chamber. Through the pipe 7 is adapted to be delivered molten metal including lead and tin from the pump 6, the metal including lead and tin being constantly circulated through this chamber. While the pipe is shown as delivering the stream of metal including lead and tin 20 straight downward, it may be inclined at an angle so that the stream of metal will promote a stirring action of the contents in the chamber or the stream may be made to hit a baffle plate to subdivide it.

The reaction chamber as shown is supported by the framework 4 and when in operative position its lower edge will be immersed in the metal inside the kettle to a depth of about 16 inches approximately.

11 is a tank containing chlorine which is led by a pipe 12 to a manifold or bustle pipe 13 which distributes the chlorine to a number of small feed pipes 14. These chlorine pipes are composed of special nickel, molybdenum, chromium, iron alloy tubes, preferably the alloy known as Hastelloy "C", which is resistant to chlorine and lead and tin chlorides at temperatures of the order of 1000° F. The tubes are approximately  $\frac{3}{8}$ " inside diameter when the dimensions given herein for other parts of the apparatus are employed. These tubes are protected by graphite tubes 14a which are slipped over them, the graphite extending the entire length of the tubes inside the reaction chamber. The graphite tubes 45 are held in place about the steel tubes by a cement 14b consisting of silica sand, finely ground brick and high alumina cement or sodium silicate. These chlorine pipes extend from the bustle pipe through the cover of the reaction chamber and being of sufficient length so that when the reaction chamber is positioned about 16 inches below the surface of the metal, as indicated above, the lower ends of these chlorine pipes are about 3 to 5 inches below the surface 50 of the metal bath inside the reaction chamber. They surround the central space in the reaction chamber. The bottom edge 15 of the reaction chamber is about 13 inches below the outlets of the chlorine pipes 14. With these dimensions 55 the diameter of the reaction chamber is approximately 29 inches and its height approximately 31 inches and the length of the chlorine tubes from the cover to their point of discharge in the reaction chamber is about 18 inches. The dimensions are given because for the embodiment shown I have obtained excellent results by having the parts proportioned as indicated, although the invention of course is not restricted to such dimensions. These dimensions have 70 been worked out to give a practical reaction

chamber. They are such as to provide a proper working depth of lead chloride and stannous chloride but to minimize the quantity of chlorides required for the operation by confining such chlorides in a small space. This is an important consideration because at the end of the operation the amount of chlorides formed in order to carry out the detinning operation is kept at a minimum and consequently the amount of pure metals recovered is correspondingly larger. I have found that it is important to maintain a sufficient depth of metal chlorides in the reaction chamber so that with a pressure of 3 to 5 lbs., or perhaps a little more, of chlorine gas as I prefer to use, there is a sufficient depth of chlorides to react efficiently with the chlorine and metallic lead and tin entering the chamber so as to avoid use of an excessive quantity of salt layer. The dimensions of the chamber are also such that the amount of surface exposed to the corrosive action of the chlorine and molten chlorides is about as small as could be satisfactorily employed for practical working conditions.

Each of the chlorine feed pipes is connected with the bustle pipe by a T connection in which is provided a cock 16 in order to regulate the individual flow through its feed pipe. The upper end of each chlorine pipe is provided with a plug 16a, which may be removed in order to clean out the pipe if and when necessary. The numeral 17 represents control valves and a flow meter for regulating the amount of chlorine passing to the bustle pipe 13 and thence into the chlorine pipes 14. This assembly serves to deliver chlorine gas in a number of fine streams under controlled conditions.

18 represents a pipe for conducting tin tetrachloride formed in the reaction chamber away therefrom and into a pre-cooler 19, which is adapted to cool the gases and precipitate any entrained stannous and lead chloride prior to the gases reaching the water-cooled condenser 20 in which the tin tetrachloride is condensed to a liquid which is collected in the container 21 supported therebelow. 22 is a pipe conducting the non-condensable portion of gas passing from 20, and which usually consists of chlorine, to a washing tower 23, which may be filled with a packing material through which dilute caustic soda solution is circulated by the system composed of a sump tank 24 where the caustic soda, after passing through the tower, collects and from which it is pumped by the motor-operated pump 25 and returned to the top of the washing tower by the pipe 26. The apparatus including the pipe 22 and washing tower 23 is not an essential part of the equipment. It is provided to catch any volatile products passing beyond the condenser 20 due to improper operation of the process.

27 is a motor-operated fan connected to the top of the washing tower 23 which serves to keep the entire gas system from reaction chamber to and including the washer, under a slight vacuum.

The operation of the apparatus shown in Figs. 1 to 4 is briefly as follows. The metal alloy or other metal mass containing lead and tin, with or without other ingredients, is melted in the kettle 1 and heated to the temperature employed in operating the process as later described. The pump 6 is started to circulate the molten lead tin through the reaction chamber. Simultaneously chlorine gas at a measured rate is allowed to flow into the molten metal from the chlorine

tank 11 through the bustle pipe 13 and chlorine feed pipes. Tin tetrachloride is formed in the reaction chamber and volatilized. The vapor leaves the reaction chamber by means of the pipe 18, passes through the pre-cooler 19 where occasionally small amounts of stannous and lead chloride are caught. The cooled tin tetrachloride vapor enters the condenser 20 where it is condensed to a liquid, and is accumulated in the container 21 for subsequent use. If any tin tetrachloride is not condensed or if any chlorine gas should not be consumed in the reaction chamber and pass along with the tin tetrachloride, these materials then pass into the washing system, which is provided as a precautionary measure, passing in at the bottom of the tower 23 where the gases are washed with circulating dilute caustic soda.

In Fig. 5 there is shown a modified form of apparatus comprising two kettle settings. Kettle 28 is preferably much larger than kettle 29. This apparatus is devised in order that a constant level may be maintained in kettle 29 during the operation. It will be understood of course that in operating, for example as in Fig. 1, the mass of molten material in the kettle 1 gradually becomes lower due to the removal of tin as tetrachloride therefrom. Such lowering of the molten metal may be compensated for by feeding fresh metal into the pot during the early period of treatment, but this should be discontinued if the greater part of the tin is to be separated as tin tetrachloride, if the operation is to be conducted economically. In addition it would be difficult, if not impossible, to raise and lower the reaction chamber, because of the various feed and delivery pipes connected to it, in order to keep it properly immersed in the shrinking bath if no new metal is added thereto. It is important that the relation of the tips of the chlorine feed pipes with the metal and chloride bath be maintained substantially as indicated above and if there is any substantial deviation the smooth progress of the reaction may be interrupted.

Accordingly I have provided in Fig. 5 an apparatus in which a constant level is maintained in the kettle 29. In this latter kettle the reaction chamber with its outer wall 8, chlorine pipes 14, bustle pipe 13 and other associated parts are the same as described in Fig. 1, and are supported by a casting 30 on the top of the kettle 29. This casting is preferably solid and provides a cover for the kettle 29. The kettle 28, however, contains the pump 6 and pipe 7 leading therefrom into the reaction chamber. The pump 6 is supported by a casting 31 supported on the edges of the kettle. A pipe 31a serves to circulate the molten metal between the kettles 28 and 29. When the metal rises above the desired height in kettle 29, it flows over into kettle 28. Burners 32 and 33 may be introduced through the brick walls of the kettle supports 2 and either or both kettles 28 and 29 may be heated, if desired.

The modification shown in Fig. 7 is similar to that shown in Fig. 5, but kettle 28 in this instance is replaced by a furnace 34, which has an outside bay 35 communicating with the interior, which bay contains a limited quantity of molten metal and in which bay the pump 6 is placed delivering molten metal by pipe 7 to the reaction chamber. The kettle 29 is supported on a kettle base which in turn is elevated on a steel structure 36. The kettle is supported at suffi-

cient height so that it is above the furnace 34 and so that an overflow pipe 37 will remove molten metal from the kettle 29 and deposit it in the furnace 34 when the metal in kettle 29 rises above the desired level.

The operation of the apparatus shown in Figs. 5 and 7 is similar to that shown in Fig. 1.

A still further modification is shown in Fig. 6 to provide a substantially continuous process. In this instance three kettles 38, 39 and 40 are provided. The center kettle 38 corresponds to the kettle 1 in Fig. 1 and this kettle operates alternately with either kettle 39 or kettle 40. Some time may be lost in heating up a bath of metal to 1000-1050° F. which is the preferred temperature for detinning according to the process described below. Considerable time is also lost in cooling the metal bath after detinning so that it may be cast. By the arrangement shown in Fig. 6 practically continuous operation may be maintained. While metal in kettle 40 is being detinned, the metal in 39 is being cooled, cast and a new lot introduced, melted and brought up to the temperature above mentioned. The reaction chamber is situated in kettle 38 and with its associated parts is substantially the same as that shown in Fig. 5, being supported by a solid casting which serves as a cover for the kettle 38. Only a single pump 6 may be employed and when it has finished its operation in one kettle, 40 for example, it may be detached and transferred to the other kettle 39 for operation. Overflow pipes 41 and 42, provided respectively with stoppers 43 and 44, extend from the kettle 38 and deliver into the adjacent kettles, pipe 41 delivering into kettle 40 and pipe 42 delivering into kettle 39. The operation of this embodiment is as follows. Metal is charged for instance into kettle 39, heated to a process temperature, pumped through pipe 7 and delivered into the reaction chamber. Chlorine is delivered from its source through the bustle pipe 13 and chlorine pipes 14 into the reaction chamber and stannic chloride passes oil through pipe 18 through the condensing system shown in Fig. 1. During the process the pump 6 is delivering the molten metal as stated through the pipe 7 to the reaction chamber and the overflow pipe 41 being open by removal of its stopper 43, metal overflows from the kettle 38 into the kettle 40 and then is again returned by the pump. Prior to the completion of the detinning of the metal in 40, another charge of metal is placed in kettle 39 and heated up to process temperature. When detinning is completed in 40 the pump 6 with its piping 7 is shifted to kettle 39 and the process of detinning similar to that described in connection with kettle 40 is carried on here, but at this time the overflow pipe 41 is closed by stopper 43 so that the overflow occurs from pipe 42, its stopper 44 having been removed. While the detinning is occurring in kettle 39, the detinned material in 40 is cooling and being cast. After the detinning in kettle 39, the process then proceeds in 40 once more. In other words the kettles 39 and 40 are alternately used for the heating and detinning operation and then for the cooling operation.

The process described below may be conveniently carried out in the apparatus above described. I have found in accordance with my invention that when chlorine is injected into a molten lead-tin mixture or alloy with or without antimony, lead chloride and stannous chloride

are formed and these salts will float to the surface. The reaction involved is:



5. If further chlorine comes in contact with these salts—lead chloride and stannous chloride, there will be formed stannic chloride which is volatile at about 238° F., and the temperature of the lead chloride and stannous chloride being above this 10 point, the stannic chloride will be volatilized and is removed from the mass. As the stannic chloride is removed, further quantities of stannous chloride must be formed, which in turn reacts with a further quantity of chlorine to produce 15 stannic chloride.

I have found in accordance with my invention that it is important to keep the five chief reacting materials involved in the production of tin tetrachloride from mixtures containing lead and 20 tin, namely tin, lead, stannous chloride, lead chloride and chlorine, all in active contact with one another. It is important to have a large 25 surface of chlorine exposed to the reacting materials. It is also important to keep the metal salts in constant agitation so that the other three 30 reacting materials may come in contact with them. If ordinary mechanical agitators are employed, it is difficult to keep any agitation equipment in operation because of the terrific attack 35 by the chloride at the elevated temperature, which I prefer to be in excess of 1000° F.

I have found that by introducing chlorine into a reaction chamber in contact with molten metal containing tin and lead and perhaps other ingredients, forming a salt layer containing lead and stannous chloride and discharging a stream of molten metal containing lead, tin and perhaps other ingredients through this salt layer, that I can satisfactorily produce tin tetrachloride. 40 Under proper conditions which will be given in greater detail below, the process can be conducted economically and efficiently. Although I do not wish to be bound by the following explanation, there appears to occur under these conditions the 45 establishment of an equilibrium or balance between the components lead chloride, stannous chloride, lead and tin, which balance is being continuously upset by the introduction of further quantities of chlorine. Chlorine reacts with the 50 stannous chloride to form tin tetrachloride which is then volatilized. The equilibrium being upset is then restored by the formation of stannous chloride by reaction of tin with lead chloride. The reactions mentioned are as follows:



55. The affinity of the different metals and their lower chlorides or chlorine are such that very little antimony or arsenic, if any be present, goes into the salt layer and the resulting tin tetrachloride contains usually not more than 60 fractions of percents of either. The heat of the above reactions involving the production of tin tetrachloride and stannous chloride tends to raise the temperature in the reaction chamber. The 65 temperature in this chamber should be maintained preferably in a range of about 1000° F. to 1050° F. since if it rises much above this point stannous chloride which has a boiling temperature of approximately 1150° F. may pass off with the tin tetrachloride. The molten metal which is 70 pumped through the reaction chamber is or-

dinarily below the temperature of the chlorinating zone. Even though the temperature of the salt layer in the reaction chamber tends to be higher than the molten bath of lead, tin and other metals with which it is in contact, nevertheless the temperature of this molten bath because of the large volume of metal therein is lower than that in the reaction chamber and furthermore a certain amount of cooling of this molten metal occurs during the pumping operation so that the molten metal delivered by the pump into the reaction chamber is at a temperature where it aids in maintaining the temperature of the reaction chamber within the desired limits. Accordingly after the chlorinating reaction has started in the reaction chamber, it is ordinarily not necessary to apply heat to the kettle to raise or maintain the temperature of the metal, but if this should be necessary of course the kettle may be heated by the burner shown thereunder in the above embodiments of the apparatus.

The following is a description of an embodiment of the process as I now prefer to practice it: A charge of material containing lead and tin usually in the form of a lead alloy of about 80,000 lbs. containing about 12% tin, is heated to 1000–1050° F. for example in the kettle 1 shown in Fig. 1. Lead chloride has a melting point of approximately 930° F. and I regard it as important to keep the temperature somewhat above this melting point in order to avoid plugging the pipes 14 through which the chlorine gas emerges. The molten alloy is circulated from the kettle 1 through the pump 6 and through the reaction chamber and chlorine is fed into the reaction chamber from the tank 11. The chlorine reacts with the metal to build up a salt layer of lead chloride and stannous chloride and the molten alloy passing into the reaction chamber is discharged through this salt layer by the pump 6 at a rate of 25,000 to 40,000 lbs. per hour. The reaction chamber as noted in the description of the apparatus is suitably positioned below the surface of the molten metal. Where the diameter of the reaction chamber is about 29 inches and its height approximately 31 inches, the reaction chamber will be about 16 inches below the surface of the metal and the ends of the chlorine tubes from the cover of the reaction chamber to their point of discharge will be about 18 inches and they will terminate, therefore, about 13 inches from the bottom of the reaction chamber. The chlorine is delivered to the reaction chamber under a pressure of about 3 to 5 lbs. per square inch and the rate of delivery of the chlorine is controlled by the control valves and meter 17 depending on the amount of tin present in the molten metal. The smaller the amount of tin the less the chlorine conveyed to the reaction chamber. Usually at the beginning of the operation when the metal contains the initial quantity, 12% of tin, 350 lbs. of chlorine per hour are used and the amount is then tapered down in about the following way:

| Percent tin in metal | Pounds of Cl per hour |
|----------------------|-----------------------|
| 1.5                  | 200                   |
| 0.75                 | 100                   |
| 0.50                 | 50                    |

During the first three or four hours of feeding chlorine gas, substantially no tin tetrachloride is 75

produced which seems to indicate that during this period the chlorine is consumed in producing a layer of stannous chloride and lead chloride in the reaction chamber.

- 5 Under the above conditions a layer of lead chloride and stannous chloride forms and displaces the alloy in the reaction chamber and the ends of the chlorine feed pipes become submerged in the salt layer, consisting of lead chloride and 5 stannous chloride. The depth of the chloride layer formed is such that with chlorine gas at 3 to 5 lbs. per sq. inch the chlorine will penetrate and react as far as the bottom of the layer but will not emerge substantially beyond it. From 10 this time on it appears that the chlorine gas entering the salt layer reacts with the stannous chloride to form a volatile tetrachloride and upon depletion of the stannous chloride in this way the reactions above mentioned to reestablish the 15 equilibrium appear to occur. When the metal left in the kettle 1 contains above 0.25% tin, the operation is considered finished as this is about the lowest content of tin that can be ordinarily obtained commercially.
- 20 25 The tin tetrachloride produced is preferably conducted to a pre-cooler 19 where any entrained liquids or high boiling liquids, which can be condensed at a higher temperature than that required for tin tetrachloride, are removed from the 25 tin tetrachloride and returned to the reaction chamber by gravity. The tin tetrachloride vapor then passes to the condenser 20 where it is condensed to a liquid and is accumulated in the container 21 for subsequent use. Any tin tetrachloride not condensed in 20 or any chlorine gas not 30 consumed in the reaction chamber and passed along with the tin tetrachloride is washed out with caustic soda solution. Very little chlorine gas in practice needs to be washed out as the 35 efficiency of chlorine absorption in the reaction chamber is high.
- 40 45 At the end of a run which ordinarily lasts two to three days depending on the original tin content of the metal being treated, there remains in the reaction chamber and floating on the metal bath about 2% of lead chloride of the original weight of alloy treated.

As the tin is eliminated as tin tetrachloride, the level of the metal bath in the kettle 1 is progressively lowered. As it is important to keep the metal level approximately constant for efficient operation, I feed in fresh quantities of metal to the kettle 1 during the run in order to maintain the original level. It is advantageous to use for this purpose metal richer in tin than the original metal so that the production of tin tetrachloride is maintained at the maximum.

I have treated compositions containing not only lead and tin but also containing from 2.5 to 19% 50 antimony and have found that the antimony contents had no adverse effects on the removal of the tin. In treating one composition which contained 8% antimony and 5% tin along with the balance lead, the lead chloride produced at the end of the 55 operation contained approximately 0.77% antimony. I have also satisfactorily operated the process on numerous lots of material containing the following ranges of materials:

|          | Per cent   |
|----------|------------|
| 70 Tin   | 1.7 to 21  |
| Bismuth  | 0 to 7     |
| Copper   | trace to 5 |
| Arsenic  | 0.1 to 4   |
| Antimony | 8 to 26    |

and the balance lead.

In accordance with my experience in practicing my invention, I have found that the best results are obtained when lead tin alloys are used which contain substantially no other ingredients or only small proportions of other ingredients which are 5 present as the raw material subjected to the process. I do not add catalysts such as sulfides, antimony or other ingredients to the raw material being treated, and I prefer to remove sulphur if it is present in the metal being treated.

The tetrachloride of tin produced by the process is remarkably pure when considering the impurity of the various compositions treated. I have found it to contain not over .04 to .92% of such impurities with 99.96% to 99.08% of tin tetrachloride. The impurities found in the tin tetrachloride will depend upon the quality of the metal being treated. The apparatus described above has been used satisfactorily in the carrying out of the various process operations described.

A process which comprises among other things the maintenance of a substantially constant level in the kettle where the reaction chamber is located may be carried out for example employing an apparatus like that shown in Fig. 5. The lead and tin are melted in the kettles 28 and 29 and the pump 6 started in kettle 28, chlorine being fed to the reaction chamber through the tubes 14. A chloride layer forms in the reaction chamber floating on the molten metal beneath. Chlorine 30 comes in contact with the chloride layer and the metal being circulated by the pump. The stream of metal passing through the chloride layer passes into the kettle 29 and then overflows through the pipe 21a into the kettle 28. Stannic chloride is removed through the pipe 18 and may be condensed as heretofore described.

A similar process may be carried out employing the apparatus shown in Fig. 7.

In carrying out a continuous process for separating tin as tetrachloride from alloys of mixtures containing tin and lead, I may employ an apparatus such as that shown in Fig. 6. Here lead is melted in the kettle 40 and pumped for example from vessel 40 through the reaction chamber in vessel 38 where it comes in contact with a plurality of streams of chlorine to form a separate layer of stannous chloride and lead chloride. The stream of molten lead passes through the layer of chlorides after it is formed and stannic chloride is removed from the reaction chamber until the quantity of tin in the molten metal is substantially reduced. Then a second mass of tin and lead is heated in the vessel 39 and circulated through the reaction chamber in contact with the streams of chlorine to form a molten chloride layer and to produce tin chloride. During this operation the metal in 40 is cooling so that it may be cast. It is removed when cool and then prior to the detinning of the material in the kettle 39 a fresh lot of tin and lead is placed in kettle 40 and heated up so that when the detinning operation ceases in kettle 39, another operation may be started on the new metal in kettle 40 so that the process is operated continuously.

While the invention has been described in detail with respect to particular preferred examples, it will be understood by those skilled in the art after understanding the invention, that various changes and further modifications may be 65 made without departing from the spirit and scope of the invention, and it is intended therefore in the appended claims to cover all such changes and modifications.

What is claimed as new and desired to be se- 75

cured by Letters Patent of the United States is:

1. In apparatus for treating metals in combination, a container for molten metal, a reaction chamber within it and near the top thereof and opening into said container, means to circulate said metal from said container through said reaction chamber and back to said container, means to maintain a layer of chlorides on top of the molten metal in said container and within said reaction chamber, and means for passing chlorine in streams into said layer of chlorides.
2. In apparatus for treating metals in combination, a container for molten metal, a reaction chamber within it and near the top thereof and opening into said container, a pump suspended in the container to circulate said metal from said container through said reaction chamber and back to said container, means to form streams of chlorine in said reaction chamber to react with said metal to form a layer of chlorides whereby when the molten metal is in the container the chlorinated metal floats thereon in the reaction chamber, the molten metal is circulated through the chlorides and the chlorine passes into the chlorides in the reaction chamber.
3. In apparatus for treating metals in combination, a container for molten metal, a reaction chamber within it and near the top thereof and opening into said container, means located near the bottom of said container to circulate said metal from said container through said reaction chamber and back to said container, a chlorine container and a passage leading therefrom to said reaction chamber, and a series of pipes in said reaction chamber to conduct the chlorine therethrough in streams and to react with said metal to form a layer of chlorides whereby when the molten metal is in the container the chlorinated metal floats thereon in the reaction chamber, the molten metal is circulated through the chlorides and the chlorine passes into the chlorinated metal in the reaction chamber.
4. In apparatus for treating metals in combination, a kettle for molten metal including lead and tin, a reaction chamber within it open at the bottom and adapted to dip into the metal and allow the metal to rise therein when the latter fills the kettle to a point near the top, said chamber being lined with material refractory to lead and tin chlorides at a temperature about 1000-1050° F., a pump in said kettle to circulate said metal from the kettle through said reaction chamber and back to said kettle, a source of chlorine delivering chlorine to said reaction chamber and a series of metal alloy tubes surrounded by graphite and passing through the refractory material to a position a short distance above the lower edge of the reaction chamber, said tubes being adapted to conduct chlorine in a series of streams into an open space in the reaction chamber adapted to be partially occupied by said molten metal, whereby upon chlorine coming into contact with the molten metal in the reaction chamber a layer of chlorinated metal is formed floating on the molten metal beneath and when the molten metal is pumped from the kettle to the reaction chamber it passes through the chlorinated metal layer at the same time that the chlorine passes into contact with the stream of molten metal

delivered by the pump and the chlorinated metal in the reaction chamber.

5. In an apparatus for treating metals in combination, a source of molten metal including lead and tin, a reaction chamber in communication therewith, means to form and maintain a layer containing tin and lead chlorides in said reaction chamber, means to bring streams of chlorine in contact with said layer of chlorides, means for circulating metal from below said layer and discharging it above and into said layer, means to conduct away the volatile chloride of tin, and a condenser to condense and recover said volatilized tin.

6. In apparatus for treating metals in combination, a container for molten metal including tin, a reaction chamber near the top thereof and opening into said container, a second container for molten metal, means to circulate said metal successively through the containers and the reaction chamber, means to bring streams of chlorine in said reaction chamber into reaction with said metal to form a layer of chlorides, and to form and remove stannic chloride from the reaction chamber whereby the level of the molten metal in said first mentioned container may be maintained substantially constant regardless of the removal of tin as tin tetrachloride from the molten metal.

7. In a continuous apparatus for separating tin from alloys or mixtures containing tin and lead in combination, a reaction kettle having a reaction chamber located therein, a second kettle communicating therewith, and a third kettle communicating with said reaction kettle, said second and third kettles being adapted to be alternatively put in communication with said reaction kettle, a pump adapted to be located alternatively in the second or third kettle for circulating molten metal from for example the second kettle in which it is located through the reaction chamber and to return it to such kettle, and alternatively to be placed in the third kettle to circulate metal through it and the reaction kettle and reaction chamber, and a source of chlorine adapted to supply chlorine to the reaction chamber continuously, whereby two lots of metal may be successively acted upon in the reaction chamber and after one lot has been treated it may be allowed to cool for casting while the second lot is being passed through the reaction chamber.

8. In an apparatus for treating metals in combination, means to maintain a layer of tin and lead chlorides on top of a molten metal bath containing tin and lead, means for passing chlorine into said layer of chlorides, and means for circulating metal from below said layer and discharging it on or into said layer.

9. A reaction chamber for the separation of metallic constituents of metals or alloys of the nature of lead and tin by a treatment of vapor of halogen consisting of a hollow metallic body suspended in the molten metal or alloy in such a manner that an efficient seal is obtained, distributing ducts penetrating said hollow metallic body and ending in openings in a substantially non-metallic refractory lining adjoining said hollow metallic body, an opening above the level of the molten metal or alloy for the admission of same into said reaction chamber and an opening for the exit of reaction products.

ELMER H. GREENBERG.